



US007972657B2

(12) **United States Patent**  
**Schlichting et al.**

(10) **Patent No.:** **US 7,972,657 B2**  
(45) **Date of Patent:** **Jul. 5, 2011**

(54) **SILICATE RESISTANT THERMAL BARRIER COATING WITH ALTERNATING LAYERS**

(75) Inventors: **Kevin W. Schlichting**, South Glastonbury, CT (US); **David A. Litton**, West Hartford, CT (US); **Michael J. Maloney**, Marlborough, CT (US); **Melvin Freling**, West Hartford, CT (US); **John G. Smeggil**, Simsbury, CT (US); **David B. Snow**, Glastonbury, CT (US)

(73) Assignee: **United Technologies Corporation**, Hartford, CT (US)

(\*) Notice: Subject to any disclaimer, the term of this patent is extended or adjusted under 35 U.S.C. 154(b) by 0 days.

(21) Appl. No.: **12/697,345**

(22) Filed: **Feb. 1, 2010**

(65) **Prior Publication Data**

US 2010/0136241 A1 Jun. 3, 2010

**Related U.S. Application Data**

(62) Division of application No. 11/516,389, filed on Sep. 6, 2006, now Pat. No. 7,722,959.

(51) **Int. Cl.**  
**B05D 7/00** (2006.01)

(52) **U.S. Cl.** ..... 427/419.2; 427/419.3

(58) **Field of Classification Search** ..... None  
See application file for complete search history.

(56) **References Cited**

U.S. PATENT DOCUMENTS

|              |         |               |
|--------------|---------|---------------|
| 6,106,959 A  | 8/2000  | Vance et al.  |
| 6,294,260 B1 | 9/2001  | Subramanian   |
| 6,808,761 B2 | 10/2004 | Chaput et al. |

FOREIGN PATENT DOCUMENTS

|    |            |         |
|----|------------|---------|
| EP | 1357201 A1 | 10/2003 |
| EP | 1806431 A2 | 7/2007  |
| EP | 1811060 A2 | 7/2007  |
| EP | 1811061 A2 | 7/2007  |
| EP | 1889949 A2 | 2/2008  |
| WO | 0009778 A1 | 2/2000  |

*Primary Examiner* — Timothy M Speer

(74) *Attorney, Agent, or Firm* — Bachman & LaPointe, P.C.

(57) **ABSTRACT**

A thermal barrier coating system for use on a turbine engine component which reduces sand related distress is provided. The coating system comprises at least one first layer of a stabilized material selected from the group consisting of zirconia, hafnia, and titania and at least one second layer containing at least one of oxyapatite and garnet. Where the coating system comprises multiple first layers and multiple second layers, the layers are formed or deposited in an alternating manner.

**11 Claims, 1 Drawing Sheet**





## SILICATE RESISTANT THERMAL BARRIER COATING WITH ALTERNATING LAYERS

### CROSS REFERENCE TO RELATED APPLICATION(S)

This application is a divisional application of allowed U.S. Patent Application Ser. No. 11/516,389, filed Sep. 6, 2006, entitled SILICATE RESISTANT THERMAL BARRIER COATING WITH ALTERNATING LAYERS.

### BACKGROUND OF THE INVENTION

#### (1) Field of the Invention

The present invention relates to a thermal barrier coating having alternating layers of oxyapatite and/or garnet and yttria-stabilized zirconia which can be applied to a turbine engine component, to a method for forming the coating, and to a turbine engine component having the coating.

#### (2) Prior Art

The degradation of turbine airfoils due to sand related distress of thermal barrier coatings is a significant concern with all turbine engines used in a desert environment. This type of distress can cause engines to be taken out of operation for significant repairs.

Sand related distress is caused by the penetration of fluid sand deposits into the thermal barrier coatings which leads to spallation and accelerated oxidation of any exposed metal.

### SUMMARY OF THE INVENTION

In accordance with the present invention, there is provided a coating system which reduces sand related distress on turbine engine components. The coating system broadly comprises alternating layers of oxyapatite and/or garnet and a stabilized zirconia, hafnia, or titania material. Herein, garnet refers broadly to an oxide with the ideal formula of  $A_3B_2X_3O_{12}$ , where A comprises at least one of the metals selected from the group consisting of  $Ca^{+2}$ ,  $Gd^{+3}$ ,  $In^{+3}$ ,  $Mg^{+2}$ ,  $Na^+$ ,  $K^+$ ,  $Fe^{+2}$ ,  $La^{+2}$ ,  $Ce^{+2}$ ,  $Pr^{+2}$ ,  $Nd^{+2}$ ,  $Pm^{+2}$ ,  $Sm^{+2}$ ,  $Eu^{+2}$ ,  $Gd^{+2}$ ,  $Tb^{+2}$ ,  $Dy^{+2}$ ,  $Ho^{+2}$ ,  $Er^{+2}$ ,  $Tm^{+2}$ ,  $Yb^{+2}$ ,  $Lu^{+2}$ ,  $Sc^{+2}$ ,  $Y^{+2}$ ,  $Ti^{+2}$ ,  $Zr^{+2}$ ,  $Hf^{+2}$ ,  $V^{+2}$ ,  $Ta^{+2}$ ,  $Cr^{+2}$ ,  $W^{+2}$ ,  $Mn^{+2}$ ,  $Tc^{+2}$ ,  $Re^{+2}$ ,  $Fe^{+2}$ ,  $Os^{+2}$ ,  $Co^{+2}$ ,  $Ir^{+2}$ ,  $Ni^{+2}$ ,  $Zn^{+2}$ , and  $Cd^{+2}$ ; where B comprises at least one of the metals selected from the group consisting of  $Zr^{+4}$ ,  $Hf^{+4}$ ,  $Gd^{+3}$ ,  $Al^{+3}$ ,  $Fe^{+3}$ ,  $La^{+2}$ ,  $Ce^{+2}$ ,  $Pr^{+2}$ ,  $Nd^{+2}$ ,  $Pm^{+2}$ ,  $Sm^{+2}$ ,  $Eu^{+2}$ ,  $Gd^{+2}$ ,  $Tb^{+2}$ ,  $Dy^{+2}$ ,  $Ho^{+2}$ ,  $Er^{+2}$ ,  $Tm^{+2}$ ,  $Yb^{+2}$ ,  $Lu^{+2}$ ,  $In^{+3}$ ,  $Sc^{+2}$ ,  $Y^{+2}$ ,  $Cr^{+3}$ ,  $Sc^{+3}$ ,  $Y^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; where X comprises at least one of the metals selected from the group consisting of  $Si^{+4}$ ,  $Ti^{+4}$ ,  $Al^{+4}$ ,  $Fe^{+3}$ ,  $Cr^{+3}$ ,  $Sc^{+3}$ ,  $Y^{+3}$ ,  $V^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; and where O is oxygen. Furthermore, limited substitution of S, F, Cl, and OH for oxygen in the above formula is possible in this compound as well, with a concomitant change in the numbers of A, B, and X type elements in the ideal formula, to maintain charge neutrality. Herein, oxyapatite refers broadly to



(II)

where A comprises at least one of the metals selected from the group consisting of  $Ca^{+2}$ ,  $Mg^{+2}$ ,  $Fe^{+2}$ ,  $Na^+$ ,  $K^+$ ,  $Gd^{+3}$ ,  $Zr^{+4}$ ,  $Hf^{+4}$ ,  $Y^{+2}$ ,  $Sc^{+2}$ ,  $Sc^{+3}$ ,  $In^{+3}$ ,  $La^{+2}$ ,  $Ce^{+2}$ ,  $Pr^{+2}$ ,  $Nd^{+2}$ ,  $Pm^{+2}$ ,  $Sm^{+2}$ ,  $Eu^{+2}$ ,  $Gd^{+2}$ ,  $Tb^{+2}$ ,  $Dy^{+2}$ ,  $Ho^{+2}$ ,  $Er^{+2}$ ,  $Tm^{+2}$ ,  $Yb^{+2}$ ,  $Lu^{+2}$ ,  $Sc^{+2}$ ,  $Y^{+2}$ ,  $Ti^{+2}$ ,  $Zr^{+2}$ ,  $Hf^{+2}$ ,  $V^{+2}$ ,  $Ta^{+2}$ ,  $Cr^{+2}$ ,  $W^{+2}$ ,  $Mn^{+2}$ ,  $Tc^{+2}$ ,  $Re^{+2}$ ,  $Fe^{+2}$ ,  $Os^{+2}$ ,  $Co^{+2}$ ,  $Ir^{+2}$ ,  $Ni^{+2}$ ,  $Zn^{+2}$ , and  $Cd^{+2}$ ; where B comprises at least one of the metals selected from the group consisting of  $Gd^{+3}$ ,  $Y^{+2}$ ,  $Sc^{+2}$ ,  $In^{+3}$ ,  $Zr^{+4}$ ,  $Hf^{+4}$ ,  $Cr^{+3}$ ,  $Sc^{+3}$ ,

**2**  
 $Y^{+3}$ ,  $V^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; where X comprises at least one of the metals selected from the group consisting of  $Si^{+4}$ ,  $Ti^{+4}$ ,  $Al^{+4}$ ,  $Cr^{+3}$ ,  $Sc^{+3}$ ,  $Y^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; and where O is oxygen. Furthermore, limited substitution of S, F, Cl, and OH for oxygen in the above formula is possible in this compound as well, with a concomitant change in the numbers of A, B, and X type elements in the ideal formula, to maintain charge neutrality.

Further, in accordance with the present invention, a turbine engine component is provided which broadly comprises a substrate and a thermal barrier coating comprising alternating layers of oxyapatite and/or garnet and a stabilized zirconia, hafnia, or titania material.

Still further, in accordance with the present invention, there is provided a method for forming a coating system which reduces sand related distress, which method broadly comprises the steps of providing a substrate and forming a coating having alternating layers of oxyapatite and/or garnet and a stabilized zirconia, hafnia, or titania material.

Other details of the silicate resistant thermal barrier coating with alternating layers of the present invention, as well as other objects and advantages attendant thereto, are set forth in the following detailed description and the accompanying drawings wherein like reference numerals depict like elements.

### BRIEF DESCRIPTION OF THE DRAWINGS

The FIGURE is a schematic representation of a substrate having a silicate resistant thermal barrier coating in accordance with the present invention.

### DETAILED DESCRIPTION OF THE PREFERRED EMBODIMENT(S)

It has been discovered that certain coatings react with fluid sand deposits and a reaction product forms that inhibits fluid sand penetration into the coating. The present invention relates to a coating system for a component, such as a turbine engine component, which takes advantage of this discovery.

Referring now to the FIGURE, there is shown a substrate 10 which may be a portion of a turbine engine component, such as an airfoil or a platform. The substrate 10 may be formed from any suitable metallic material known in the art such as a nickel based superalloy, a cobalt based alloy, a molybdenum based alloy, a niobium based alloy, or a titanium based alloy. Alternatively, the substrate 10 may be a ceramic based material or a ceramic matrix composite material.

The FIGURE schematically shows an optional layer 11 deposited on the substrate that consists of an oxidation resistant bondcoat. The bondcoat may be formed from any suitable oxidation resistant coating known in the art such as NiCoCrAlY or (Ni,Pt)Al bondcoats, i.e. a simple NiAl CrPtAl bondcoat. Alternatively, and especially for ceramic substrates, the bondcoat material could consist of  $MoSi_2$ , or  $MoSi_2$  composites containing  $Si_3N_4$  and/or SiC. Furthermore, the bondcoat material could consist of elemental Si. The bondcoat layer could be formed on the substrate by any suitable technique known in the art, including air plasma spraying, vacuum plasma spraying, pack aluminizing, over-the-pack aluminizing, chemical vapor deposition, directed vapor deposition, cathodic arc physical vapor deposition, electron beam physical vapor deposition, sputtering, sol-gel, or slurry-dipping.

In accordance with the present invention, a thermal barrier coating **12** is formed on at least one surface of the substrate **10**. The thermal barrier coating **12** comprises a first layer **14** of a stabilized zirconia, hafnia, or titania material deposited onto at least one surface of the substrate **10**. Rare earth materials may be used to stabilize the zirconia, hafnia, or titania. The rare earth materials may be at least one oxide selected from the group consisting of lanthanum, cerium, praseodymium, neodymium, promethium, samarium, europium, gadolinium, terbium, dysprosium, holmium, erbium, thulium, ytterbium, lutetium, scandium, indium, and mixtures thereof. The rare earth materials may be present in an amount from 5.0 to 99 wt %, preferably 30 to 70 wt %. Alternatively, the zirconia, hafnia, or titania, may be stabilized with from about 1.0 to 25 wt %, preferably from 5.0 to 9.0 wt %, yttria. The first layer may have a thickness in the range of from 0.5 to 50 mils, preferably from 0.5 to 5.0 mils.

After the first layer **14** has been deposited, a second layer **16** of oxyapatite and/or garnet is then applied on top of the first layer **14**. The second layer **16** has a thickness from 0.5 to 50 mils, preferably from 0.5 to 5.0 mils. If the second layer contains both oxyapatite and garnet, each can be present in an amount from 5.0 to 90 wt %, preferably from 5.0 to 50 wt %.

Thereafter, this process of forming alternating layers **14** and **16** is continued until the thermal barrier coating has a desired thickness in the range of from 0.5 to 40 mils.

In a preferred embodiment of the present invention, the last or outermost layer of the thermal barrier coating **12** is an oxyapatite and/or garnet layer. The oxyapatite and/or garnet layers act as barrier to molten sand penetration into the coating.

The layers **14** and **16** may be deposited using any suitable technique known in the art. For example, each layer may be deposited using electron beam physical vapor deposition (EB-PVD) or air-plasma spray (APS). Other application methods which can be used include sol-gel techniques, slurry techniques, chemical vapor deposition (CVD), and/or sputtering.

The benefit of the present invention is a thermal barrier coating that resists penetration of molten silicate material and provides enhanced durability in environments where sand induced distress of turbine airfoils occurs. The alternating layers of oxyapatite/garnet and yttria-stabilized zirconia seal the thermal barrier coating from molten sand infiltration.

It is apparent that there has been provided in accordance with the present invention a silicate resistant thermal barrier coating with alternating layers which fully satisfies the objects, means, and advantages set forth hereinbefore. While the present invention has been described in the context of the specific embodiments thereof, other unforeseeable alternatives, modifications, and variations may become apparent to those skilled in the art having read the foregoing description. Accordingly, it is intended to embrace those alternatives, modifications, and variations as fall within the broad scope of the appended claims.

What is claimed is:

1. A method for forming a coating system on a substrate comprising the steps of:  
providing a substrate;  
forming a first layer of a stabilized material selected from the group consisting of zirconia, hafnia, and titania on at least one surface of said substrate; and  
forming a second layer containing at least one of oxyapatite and garnet over said first layer, and

depositing an additional first layer over said second layer and depositing an additional second layer of said first layer;

whereby an outermost layer of said coating system comprises a second layer.

2. The method according to claim 1, further comprising depositing additional first layers and additional second layers in an alternating manner until said coating system has a thickness in the range of from 0.5 to 40 mils.

3. The method according to claim 1, wherein said first layer forming step comprises depositing a layer of a material selected from the group consisting of zirconia, hafnia, and titania stabilized with a rare earth material comprises at least one oxide selected from the group consisting of lanthanum, cerium, praseodymium, neodymium, promethium, samarium, europium, gadolinium, terbium, dysprosium, holmium, erbium, thulium, ytterbium, lutetium, scandium, indium and mixtures thereof.

4. The method according to claim 1, wherein said first layer forming step comprises depositing a layer of a material selected from the group consisting of zirconia, hafnia, and titania stabilized with yttria.

5. The method according to claim 1, wherein said second layer forming step comprises depositing a layer of oxyapatite.

6. The method according to claim 1, wherein said second layer forming step comprises depositing a layer of garnet.

7. The method according to claim 1, wherein said substrate providing step comprises providing a turbine engine component formed from a metallic material selected from the group consisting of a nickel based superalloy, a cobalt based alloy, a molybdenum based alloy, a niobium based alloy, a titanium based alloy, a ceramic based material, and a ceramic matrix composite substrate.

8. The method according to claim 1, wherein said second layer forming step comprises forming a layer containing an oxyapatite having the formula  $A_4B_6X_6O_{26}$  where A comprises at least one of the metals selected from the group consisting of is  $Ca^{+2}$ ,  $Mg^{+2}$ ,  $Fe^{+2}$ ,  $Na^+$ ,  $K^+$ ,  $Gd^{+3}$ ,  $Zr^{+4}$ ,  $Hf^{+4}$ ,  $Y^{+2}$ ,  $Sc^{+2}$ ,  $Sc^{+3}$ ,  $In^{+3}$ ,  $La^{+2}$ ,  $Ce^{+2}$ ,  $Pr^{+2}$ ,  $Nd^{+2}$ ,  $Pm^{+2}$ ,  $Sm^{+2}$ ,  $Eu^{+2}$ ,  $Gd^{+2}$ ,  $Tb^{+2}$ ,  $Dy^{+2}$ ,  $Ho^{+2}$ ,  $Er^{+2}$ ,  $Tm^{+2}$ ,  $Yb^{+2}$ ,  $Lu^{+2}$ ,  $Sc^{+2}$ ,  $Y^{+2}$ ,  $Ti^{+2}$ ,  $Zr^{+2}$ ,  $Hf^{+2}$ ,  $V^{+2}$ ,  $Ta^{+2}$ ,  $Cr^{+2}$ ,  $W^{+2}$ ,  $Mn^{+2}$ ,  $Tc^{+2}$ ,  $Re^{+2}$ ,  $Fe^{+2}$ ,  $Os^{+2}$ ,  $Co^{+2}$ ,  $Ir^{+2}$ ,  $Ni^{+2}$ ,  $Zn^{+2}$ , and  $Cd^{+2}$ ; where B comprises at least one of the metals selected from the group consisting of  $Gd^{+3}$ ,  $Y^{+2}$ ,  $Sc^{+2}$ ,  $In^{+3}$ ,  $Zr^{+4}$ ,  $Hf^{+4}$ ,  $Cr^{+3}$ ,  $Sc^{+3}$ ,  $Y^{+3}$ ,  $V^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; where X comprises at least one of the metals selected from the group consisting of  $Si^{+4}$ ,  $Ti^{+4}$ ,  $Al^{+4}$ ,  $Cr^{+3}$ ,  $Sc^{+3}$ ,  $Y^{+3}$ ,  $V^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; and where O is oxygen.

9. The method according to claim 1, wherein said second layer forming step comprises forming a layer containing a garnet having the formula  $A_3B_2X_3O_{12}$  where A comprises at least one of the metals selected from the group consisting of  $Ca^{+2}$ ,  $Gd^{+3}$ ,  $In^{+3}$ ,  $Mg^{+2}$ ,  $Na^+$ ,  $K^+$ ,  $Fe^{+2}$ ,  $La^{+2}$ ,  $Ce^{+2}$ ,  $Pr^{+2}$ ,  $Nd^{+2}$ ,  $Pm^{+2}$ ,  $Sm^{+2}$ ,  $Eu^{+2}$ ,  $Gd^{+2}$ ,  $Tb^{+2}$ ,  $Dy^{+2}$ ,  $Ho^{+2}$ ,  $Er^{+2}$ ,  $Tm^{+2}$ ,  $Yb^{+2}$ ,  $Lu^{+2}$ ,  $Sc^{+2}$ ,  $Y^{+2}$ ,  $Ti^{+2}$ ,  $Zr^{+2}$ ,  $Hf^{+2}$ ,  $V^{+2}$ ,  $Ta^{+2}$ ,  $Cr^{+2}$ ,  $W^{+2}$ ,  $Mn^{+2}$ ,  $Tc^{+2}$ ,  $Re^{+2}$ ,  $Fe^{+2}$ ,  $Os^{+2}$ ,  $Co^{+2}$ ,  $Ir^{+2}$ ,  $Ni^{+2}$ ,  $Zn^{+2}$ , and  $Cd^{+2}$ ; where B comprises at least one of the metals selected from the group consisting of  $Zr^{+4}$ ,  $Hf^{+4}$ ,  $Gd^{+3}$ ,  $Al^{+3}$ ,  $Fe^{+3}$ ,  $La^{+2}$ ,  $Ce^{+2}$ ,  $Pr^{+2}$ ,  $Nd^{+2}$ ,  $Pm^{+2}$ ,  $Sm^{+2}$ ,  $Eu^{+2}$ ,  $Gd^{+2}$ ,  $Tb^{+2}$ ,  $Dy^{+2}$ ,  $Ho^{+2}$ ,  $Er^{+2}$ ,  $Tm^{+2}$ ,  $Yb^{+2}$ ,  $Lu^{+2}$ ,  $In^{+3}$ ,  $Sc^{+2}$ ,  $Y^{+2}$ ,  $Cr^{+3}$ ,  $Sc^{+3}$ ,  $Y^{+3}$ ,  $V^{+3}$ ,  $Nb^{+3}$ ,  $Cr^{+3}$ ,  $Mo^{+3}$ ,  $W^{+3}$ ,  $Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; where X comprises at least one of the metals selected from the group consisting of  $Si^{+4}$ ,  $Ti^{+4}$ ,  $Al^{+4}$ ,  $Cr^{+3}$ ,  $Sc^{+3}$ ,  $Y^{+3}$ ,  $V^{+3}$ ,  $Nb^{+3}$ ,  $Cr^{+3}$ ,  $Mo^{+3}$ ,  $W^{+3}$ ,

**5**

$Mn^{+3}$ ,  $Fe^{+3}$ ,  $Ru^{+3}$ ,  $Co^{+3}$ ,  $Rh^{+3}$ ,  $Ir^{+3}$ ,  $Ni^{+3}$ , and  $Au^{+3}$ ; and where O is oxygen.

**10.** The method according to claim **1**, further comprising forming a bondcoat on said substrate.

**11.** The method according to claim **10**, wherein said bondcoat forming step comprises forming said bondcoat from at

**6**

least one material selected from the groups consisting of  $NiCoCrAlY$ ,  $NiAl$ ,  $PtAl$ ,  $MoSi_2$ , a  $MoSi_2$  composite containing  $Si_3Ny$  and/or  $SiC$ , and  $Si$ .

\* \* \* \* \*